

L. B. BREWSTER AND F. WEISEHAN.

PROCESS OF WELDING.

APPLICATION FILED DEC. 7, 1917.

1,327,267.

Patented Jan. 6, 1920.



Fig. 1.



Fig. 2.

Inventors.

Leon B. Brewster and  
Frank Weisihan  
By Thurston & Koen  
Atty's.

# UNITED STATES PATENT OFFICE.

LEON B. BREWSTER AND FRANK WEISEHAN, OF CLEVELAND, OHIO, ASSIGNEES TO THE FERRO MACHINE AND FOUNDRY COMPANY, OF CLEVELAND, OHIO, A CORPORATION OF OHIO.

## PROCESS OF WELDING.

1,327,267.

Specification of Letters Patent.

Patented Jan. 6, 1920.

Application filed December 7, 1917. Serial No. 205,926.

*To all whom it may concern:*

Be it known that we, LEON B. BREWSTER and FRANK WEISEHAN, citizens of the United States, and residents, respectively, 5 of Cleveland, in the county of Cuyahoga and State of Ohio, and Cleveland, in the county of Cuyahoga and State of Ohio, have invented a certain new and useful Improvement 10 in Processes of Welding, of which the following is a full, clear, and exact description.

This invention relates to a process or method by which one metal may be deposited on another, and the deposited metal 15 is made to adhere to the metal on which it is deposited.

The process is more particularly adapted and intended for use in the filling of cavities which may occur in castings or other 20 metal objects. Generally speaking, the invention may be said to comprise the steps in the process more particularly set forth in the claims.

Reference should be had to the accompanying drawings forming a part of this 25 specification, in which Figure 1 illustrates an elevation and more or less diagrammatic arrangement of a casting and apparatus for carrying out the invention; Fig. 2 is a sectional elevation through the holder for the wire electrode.

The problem of depositing metal in cavities that may occur in castings of various metals, more particularly cast iron, due to 30 a blow hole or sand flaw in the casting, has been a very vexing one. This has arisen not so much because of the difficulty of depositing metal in such a blow hole, but because of the fact that by such processes as have 35 been tried, and in fact, by such processes with which we are familiar, the metal deposited is exceedingly hard, much harder than the metal of the body of the casting itself. Therefore, when the casting is machined, the exceedingly hard spot of metal 40 which has thus been deposited offers greater resistance to the cutting of a cutting tool than the surrounding metal, and the effect is that the cutting tool usually jumps the hard spot of metal, thereby resulting in an 45 imperfect machine.

By the process which will be herein described metal may be deposited in such a cavity, caused to adhere to the metal upon which it is deposited as by a weld, and the 55 metal which is thus deposited is not hard and difficult to machine, but will be of a hardness not greater than that of the metal of the body of the casting, and therefore when the casting is machined the cutting 60 tool will operate upon the deposited metal the same as upon the metal of the casting itself.

Such an apparatus as may be employed in carrying out the process, is illustrated in 65 the drawing, in which 1 represents a casting containing a cavity which it is desired to fill with metal. The casting is mounted upon any suitable bench, but the casting should be insulated.

At 2 there is indicated a holder, preferably made of insulating material, or, in any event, care should be taken that the holder is insulated from the wire which is represented at 3. The holder is preferably a hollow holder, so that as the wire is consumed 70 it may be fed through the holder and secured therein.

The wire is secured to one terminal 4 of a circuit 4-5 and the other terminal 5 is secured to the casting in any suitable way, as by securing the wire 5 to a contact plate 75 upon which the casting rests.

The voltage and current supplied to the terminals 4-5 may be from any suitable 80 source, and of course the current will be regulated as required.

At 7 a pipe is shown which has a restriction at one end thereof and at this end hydrogen gas is ignited. The member 7 is 85 secured to a flexible tube 8, which is in turn connected with the source of hydrogen.

In using the process, the hydrogen flame is held at the point or place where the wire 90 3 is caused to contact at the casting.

In applying our process to repairing a casting which has a blow hole in it, the blow hole is cleaned out so as to remove any sand or foreign matter. The casting is directly connected to one terminal of an electric circuit, while the other terminal of the electric circuit is formed by a metallic elec- 100

trode, the metal of the electrode being fusible at the temperatures which are developed in the use of the electrode, and the metal furthermore being ductile.

5 The metal of the electrode is in wire form, the size of the wire used varying with the work which is to be done and the quantity of current which may be necessarily used in repairing the casting.

10 The current and the voltage of the current which is supplied to the circuit may vary somewhat, but in the main will not exceed 16 volts and approximately 100 amperes. This current, it will be seen, is a

15 comparatively low current.

In carrying out the process the metallic electrode with the circuit in proper condition is introduced to the bottom of the blow hole in the casting. As the metallic elec-

20 trode contacts with the bottom of the blow hole, there is a more or less imperfect contact, and the circuit which is thus closed by the contact will therefore have a very high heating effect. This heating effect is local-

25 ized, being confined to the end of the metallic electrode, and that portion of the casting which is adjacent the end of the metallic electrode. The contact of the electrode with the casting is maintained until the rise of

30 temperature is sufficient to melt the end of the electrode, which will, of course, cause the metal thus melted to flow onto the casting and there takes place a welding action between the metal which is thus melted and

35 that portion of the cavity of the casting which has been contacted by the electrode.

The actual time required to cause the melting and deposition of the metal is very short and requires but a momentary contact.

40 As soon as this has taken place, the electrode is removed, thus breaking the circuit, and care must be taken that some degree of skill is required to remove the electrode at the proper time, in order that undue quantities of the electrode may not be removed

45 or melted away.

The electrode is moved from spot to spot in the cavity and the foregoing operation repeated until the surface of the blow hole

50 is covered by a deposit of the metal of the electrode. It will thus be seen that the surface of the blow hole is covered by a number of small particles of the metal of the electrode; all of which particles are welded

55 to the particular portion of the surface of the blow hole with which the electrode contacted.

Due to the fact that the voltage and current used are of low value, the metal which

60 is thus deposited has caused a heating of that portion of the cavity only, which was contacted by the electrode.

The metal thus deposited is ductile and when once deposited a peening hammer is

65 employed to peen the metal which has been

introduced into the blow hole, thus causing the metal to be compacted, and any inequalities in the surface of the metal reduced.

The operation before described is repeated and this repetition causes a further amount of metal to be welded to the metal previously deposited in the blow hole. The metal thus deposited is again subjected to a peening and the alternate process of depositing the metal and peening is continued until the proper amount of metal has been deposited in the blow hole to completely fill and perchance a little more than fill the cavity of the casting.

By following the process which has been described, the metal thus deposited is not hard, but is comparatively soft, that is to say, it is at least as soft as the metal of the casting itself, so that upon the machining of the casting the metal which has been deposited may be removed in the machining action with the same facility as the metal of the casting.

The foregoing process has been used with considerable success for the purpose of filling blow holes in engine cylinder castings which may develop when the engine cylinder is machined. Any blow hole developed under such conditions may readily be filled by following out the foregoing process, and if, as before stated, the engine cylinder has been machined, the excess metal which may be deposited by the process described may be removed by a suitable tool, such as a file.

It is important to distinguish the process which has been described from that process by which metal from a fusible electrode is deposited upon other metal while maintaining an arc between the metal electrode and the metal object upon which the metal from the electrode is to be deposited.

Metal which is thus deposited from a fusible electrode is exceedingly hard, and renders it quite impossible to satisfactorily machine a casting which has thus been repaired.

In the process before discussed the metal is not deposited by virtue of metal which may be carried over from the electrode to the casting in the arc stream, but on the contrary, the heat which is developed for the purpose of depositing metal from the electrode is purely a heat generated by resistance and the electrode is removed when the proper heating effect has been obtained. In carrying out the foregoing process it is highly desirable to cause the deposition of the metal from the electrode under conditions which will insure against oxidation of the molten metal. This we have satisfactorily accomplished by maintaining a reducing atmosphere at the place where the electrode is touching the casting. In practice we have found a burning hydrogen atmosphere to be very satisfactory, and for

this purpose we utilize a small hydrogen burner which is held in one hand of the operator in proper position while the other hand of the operator manipulates the fusible electrode.

Having thus described our invention, what we claim is:

1. The process of depositing metal from a fusible electrode having a high temperature point of fusion upon a body of metal having a high temperature point of fusion which consists in making the metal to receive the deposited metal one terminal of a circuit, and a fusible electrode another terminal of the circuit, bringing the fusible electrode into contact with the said metal object and holding the same in contact until the heat generated by the resistance of the current passing from the electrode to the metal object causes a heating and fusion of that portion of the metal object which is directly adjacent the electrode and causes a portion of the electrode to be melted and welded to the metal object and then removing the electrode.

2. The process of depositing metal from a fusible electrode upon a metal object which consists in making the metal object one terminal of an electric circuit and the fusible electrode another terminal of said electric circuit, causing the fusible electrode to contact with the metal object and maintaining this contact while the heat due to the resistance of the contact heats and softens the metal object in that portion thereof which is contacted by the electrode, and a portion of the electrode is melted and welded to the metal object, and during this time maintaining reducing conditions at the point the welding is taking place.

3. The process of depositing metal from a fusible electrode having a high temperature point of fusion upon a metal object

also having a high temperature point of fusion which consists in making the metal object one terminal of an electric circuit and the fusible electrode the other terminal of the circuit, supplying to said circuit a current which is of low voltage and current value, causing the fusible electrode to contact with the metal object thereby causing the metal object to be heated at the point of contact by the resistance of the current due to the contact of the electrode with the metal object, and maintaining such contact until the metal object at the point adjacent the electrode is sufficiently heated and fused and metal from the electrode is melted to secure a welding action, and then removing the electrode.

4. The process of depositing metal from the fusible electrode in a cavity of a metal object, which consists in making the metal object one terminal of an electric circuit, and a fusible electrode the other terminal of the circuit, bringing the metal electrode into contact with a portion of the cavity thereby heating that portion of the metal object with which the electrode is in contact, continuing such contact until the heat developed at the point of the metal object which is contacted is sufficient to cause a welding action between that point of the metal object and metal which is melted at the end of the fusible electrode, repeating such action until the surface of the cavity is covered by deposits of metal, peening the metal which has thus been deposited, subsequently depositing additional metal upon the peened metal and in continuing such operations until the cavity is filled.

In testimony whereof, we hereunto affix our signatures.

LEON B. BREWSTER.  
FRANK WEISEHAN.